

Dec. 10, 1957

H. T. SCHREUS ET AL

2,815,760

TOBACCO SMOKE FILTER

Filed Oct. 4, 1955

Fig. 1.



Fig. 2.



Fig. 3.



Fig. 4.



Fig. 5.



Fig. 6.



Fig. 7.



BY

Bailey, Stephens & Shottig  
ATTORNEYS

1

2,815,760

## TOBACCO SMOKE FILTER

Hans Theo Schreus, Dusseldorf, and Fritz Schönhöfer,  
Wuppertal-Vohwinkel, Germany

Application October 4, 1955, Serial No. 538,479

Claims priority, application Germany December 24, 1951

13 Claims. (Cl. 131—208)

The present invention relates to an improved filter for tobacco smoke, for removing or rendering ineffective health-affecting volatile substances contained in the tobacco smoke. The new filters comprise an extended, hollow chamber or cartridge, open at both ends through which the tobacco smoke to be purified is passed and which contains means or materials for chemically binding or adsorbing health affecting volatile constituents of the tobacco smoke without destroying or removing the aroma of the tobacco smoke. The object of this invention is to provide a filter of this kind of increased efficiency. This patent application is a continuation-in-part application of our United States patent application Serial No. 327,510, filed December 23, 1952, now abandoned.

It is known to render ineffective health-affecting volatile constituents contained in the tobacco smoke by binding them to adsorbents disposed in a filter through which the smoke is passed. For this purpose, inert adsorption agents have been used, such as carbon, silica gel, finely porous filter materials or cotton wool and the like. Attempts have also been made to obviate the harmful effects of nicotine by using filter layers impregnated with acids and in addition with oxidizing agents. All these previously used substances have the disadvantage to require large filter surfaces if a good adsorption is to be obtained.

It is also known to use cation and anion exchange materials, individually as well as mixed together, as filter materials. It is true that basic and acid components of the tobacco smoke are bound in such filters. However, it has been found that the harmful substances contained in the tobacco smoke which are neither acid nor alkaline, such as e. g. aldehydes, or ketones, will nevertheless pass this type of filter. Furthermore, known filters have the great disadvantage to unfavourably influence the taste of the tobacco smoke, so that the smoker, having used it only for a short time, takes a dislike against such filters.

It has now been found that it is possible to very effectively bind health affecting components of the tobacco smoke without disadvantageously affecting its taste by using a filter which, besides the known ion exchange materials, namely cation or anion materials or both together, contains additional materials which chemically react with the harmful, nonalkaline and nonacid components of the smoke to form non-volatile compounds, thus retaining the latter in the filter.

As to the cation exchange materials, all substances known for this purpose may be used in the present invention, preferably e. g. phenolsulfonic acid resins, sulfonic acid resins on the basis of polystyrene, sulfonated phenol resins, sulfonated polystyrene resins of the lower cross-linkage type, high-capacity sulfonated polystyrene resins, such as for instance Amberlite IR-120, Amberlite XE 66-B, Amberlite IR-1 (R. Kunin, Anal. Chem. 21 89 [1949]), resins of polyacrylic acid, such as for instance Amberlite IRC-50, Amberlite XE-64 (R. Kunin and R. E. Barry, Ind. Eng. Chem. 41 1269 [1949]; I. C. Winters and R. Kunin Ibid. 460; F. X. McGarvey

2

and Thomson, Ibid. 43 741 [1951], sulfonated carbons and other substances. All of these materials are commercially known products.

Sulfonated carbon has proved to be particularly useful. Preferably, a sulfonated carbon is used which shows such a mechanical stability that when being stored or moved in the filter it will not disintegrate and will not cause any clogging of the apertures of the filter chamber nor of the filter cartridge. This sulfonated carbon should possess such a stability that a carbon particle of about 1.5 mm. in diameter will not be crushed when charged with a weight of 200 g. Furthermore, this sulfonated carbon should possess an adequate capacity of adsorption. This property may be tested by shaking for 15 minutes 1.1 g. of the sulfonated carbon in a solution consisting of 10 cc. distilled water, 1 cc. of a solution of 0.2% methyl red and 1 drop of 20% hydrochloric acid. An adequate adsorption power of the carbon is indicated by the disappearance of the red color within this period. This sulfonated carbon is known and may be obtained according to known methods. It is a commercially available cation exchange material.

As to the anion exchange materials, for instance the following substances may be used in the present invention: Quaternary ammonium bases on the basis of polystyrene, phenol-formaldehyde-amino resins, secondary amines derived from polystyrene, such as for instance Amberlite IRA-400, Amberlite IRA-401, Amberlite IRA-410, Amberlite IRA-411 (R. Kunin and F. X. McGarvey, Ind. Eng. Chem. 41 1265 [1949]; I. C. Winters and R. Kunin, Ibid. 460 [1949] and other substances. All of these substances likewise are known commercial products.

The nonacid and nonalkaline components of the tobacco smoke which exert a harmful effect are mainly carbonyl compounds, i. e. aldehydes and ketones, such as e. g. formaldehyde, acrolein, acetone, methylethylketone or a similar substance. They may be retained in the filter material by a chemical reaction with particular filter substances with formation of nonvolatile compounds. For this purpose the known difficultly volatile carbonyl reagents, such as e. g. phenylhydrazine, semicarbazide or thiosemicarbazide and their substitution products, sodium bisulfite and metabisulfites respectively, 45 may be used as filter materials. These substances may be used per se or in the form of their salts. However, it has been found that they are particularly effective in use, if they are adsorbed on the surface of porous substances. Suitably, the filter material may be prepared by dissolving the desired carbonyl reagent in a solvent and/or diluent, such as e. g. water, methyl alcohol, ethyl alcohol, acetone, ether methylenechloride, dioxane, tetrahydrofuran or similar substances and by mixing the solution with the porous material, allowing to adsorb 55 and then removing the solvent. Activated carbon, cellulose, asbestos wool, chips of plastic material, unburned earthen pellets, particles of pumice stone, paper meal, silica gel, cork, or a similar substance may be used as porous material. This porous material can be used in a great variety of shapes, such as, for example, particles, pellets, laminas, punched or pressed stoppers, powder or crystals.

The carbonyl compounds of the tobacco smoke may also be bound by means of difficultly volatile 1,2-aminoalcohols, the amino group of which contains at least one unsubstituted hydrogen atom while forming oxazolidines for instance according to the following reaction.



The following 1,2-aminoalcohols may be used in the present invention: 1-aminoethanol-2, 1-methylaminoethanol-2, 1-ethylaminoethanol-2, 1-isopropylaminoethanol-2, di-2-2'-hydroxyethylamine, 1-hydroxy-2-aminopropane, 1-aminocyclopentanol-2, 1-aminocyclohexanol-2, 1-methylaminocyclohexanol-2, 1-allylaminothiocyclohexanol-2, 1-phenyl-1-hydroxy-2-methylaminoethane, 8-hydroxy-1,2,3,4-tetrahydroquinoline, 2-hydroxypiperidine, 1-hydroxy-1,2,3,4-tetrahydroisoquinoline, 2-hydroxypyrrrolidine, glucamine, N-methylglucamine, N-ethylglucamine or a similar substance. These 1,2-aminoalcohols, too, are suitably used as filter material, after they have been adsorbed on a porous material, such as e. g. activated carbon.

Furthermore, difficultly volatile 1,2- and 1,3-diamines each amino group of which contains at least one unsubstituted hydrogen atom may also be used in order to bind the nonacid and nonalkaline components of the tobacco smoke, such as e. g. the carbonyl compounds, for instance the following reactions taking place:



or



For instance the following diamines may be used in the present invention: 1,2-ethylene diamine, methyl-2-aminoethylamine, ethyl-2-aminoethylamine, sym. dimethyl-1,2-ethylenediamine, 1,3-propylenediamine, 1-ethylamino-3-propylamine, sym.dimethyl-1,3-propylenediamine, 1,2-diaminocyclopentane, 1,2-diaminocyclohexane, or a similar substance. These diamines likewise are suitably adsorbed on porous materials, such as e. g. activated carbon, as described above and used in this form.

Any suitable amount of the carbonyl reagents may be adsorbed on the porous substance. Especially good results were obtained with porous substances containing from 0.1 to 10% by weight adsorbed upon them.

The advantage of these basic carbonyl reagents, namely of the 1,2-aminoalcohols, 1,2- and 1,3-diamines, the hydrazines and the like, resides in the fact that they may not only chemically react with the carbonyl compounds of the tobacco smoke, but being organic bases, also neutralize the acid components of the tobacco smoke, thus retaining them in the filter. Thus, they act simultaneously like the anion exchange material which may be wholly or partially replaced by them.

In order to support the neutralization of the acid components of the tobacco smoke, difficultly volatile organic bases may be additionally used which may be adsorbed on the porous material, if desired, together with the mentioned basic carbonyl reagents.

The following organic bases may be used for this purpose: triethanolamine, 2-diethylaminoethanol, 2-dibenzylaminoethanol, 1-diethylaminopropanol-3, N-dimethylglucamine, N-diethylglucamine, piperidine, N-methylpiperidine, N-benzylpiperidine or a similar substance. However, no easily volatile amines or bases should be used because they would leave the filter during the smoking process, thus unfavorably affecting the aroma.

As mentioned above the compounds used according to this invention for binding the harmful components of the tobacco smoke must be difficultly volatile, i. e. they must not be volatile or essentially volatile below a temperature of 100° C.

Suitably the filter for the tobacco smoke consists of an extended chamber which is perforated at both ends through which the smoke of burning tobacco may be drawn, and which contains the ion exchange material and

the adsorbents of the described type. This filter material can be disposed directly within a cigarette, a cigarillo, cigar or pipe without any special casing. Alternatively, it may be contained in a special casing or cartridge which is disposed anywhere at a suitable place in a hollow chamber of the cigar or cigarette holder or in the pipe, so that this casing or cartridge may be exchanged against a new one as soon as the filter material has been exhausted. These casings may be used in a great variety of shapes, such as e. g. in the form of a cylinder, ball or cone. The hollow cylinder has proved to be a special useful form.

The drawing represents a useful form of the filter casing or cartridge. The forms of the filters shown in the drawing are illustrated on an enlarged scale.

Fig. 1 represents a filter cartridge disposed in a cigarette holder.

Fig. 2 represents a central longitudinal section through the filter cartridge.

Fig. 3 represents a cross section through the removable cap of the cartridge along the line 3-3 of Fig. 2.

Fig. 4 is a cross section through the other end of the cartridge along the line 4-4 of Fig. 2.

Figs. 5 and 6 are perspective views which show particular embodiments of the sealing cap of the cartridge.

Fig. 7 represents a central longitudinal section through a preferred filter cartridge according to the invention in which the ion exchange filtering material and the filtering material which reacts with the organic carbonyl compounds, respectively, are not intermixed.

The filter cartridge may consist of materials, such as, for example, cardboard, glass, wood, metal, earth and plastic materials. Of the latter group the customary commercial products may be used, e. g. acrylic acid ester resins, acrylonitrile resins, polyvinyl chloride, urea formaldehyde resins, phenolformaldehyde resins, polyethylene products, polystyrenes or a similar substance. A filter cartridge of plastic material is well suited for the claimed purpose; it may be colorless or colored, transparent or opaque. If the filter material is colorless, it is preferable to use a colorless transparent cartridge so that the coloring of the filter material by the tobacco smoke, and thus the degree of exhaustion of the filter material effected by the tobacco smoke, will be readily recognizable. However, when using a colored filter material, such as e. g. sulfonated carbon or activated carbon charged with the described substances it is advantageous to keep the wall of the cartridge, e. g. of the hollow cylinder, opaque while one or both closure members of the cylinder, e. g. the perforated sealing cap is to consist of a transparent material. Thus, the degree of exhaustion of the filter is easily recognizable from the coloration of the material as observed through said holes contained on those parts of the cartridge where the smoke enters or leaves it.

Fig. 1 represents a cigarette holder consisting of two parts 1 and 2 which may be screwed in one another. When being screwed together members 1 and 2 form a hollow chamber which provides for receiving the filter cartridge 3, shown in detail in Figs. 2 to 6. In the present case the cartridge is a cylindrical hollow body containing a mixture of granules 9 of filtering material according to the invention which at the end adjacent to the cigarette is closed by a jammable sealing cap 4 and which on the opposite side ends in a perforated terminal disc 5. The sealing cap 4 contains a number of axial or approximately axial bore holes 6, e. g. six symmetrical bore holes which are arranged in a concentric circle and the axes of which may be differently directed, as shown e. g. in Figs. 2, 5 and 6. The terminal disc 5 which is integrally connected with or sealed to the filter cartridge 3 suitably shows a concentric aperture 7 with support stays 8, as shown in Fig. 4. The bore holes contained in the sealing cap when disposed with inclined axes as in Figs. 5 and 6 have the advantage to bring about a turbulent movement of the tobacco smoke during smoking, whereby

the filter materials contained in the cartridge are better passed and washed around them with exactly axial bore holes.

The dimensions of the cartridge may be adapted to any desired purpose of use. The following dimensions are preferred which, when compared with the measures of known cartridges, additionally allow a more fashionable form of the holders and the pipes: The external length of the cartridge, without the sealing cap, measures about 46 mm. its external diameter being about 7 mm. The sealing cap 4 measures about 7 times 3 mm. and the sealed cartridge has a total length of about 47 mm. Of course, these are only optimum dimensions for the cartridge, which, if desired, may be varied.

Suitably, the filter cartridge is disposed in the holder or pipe in such a manner that the sealing cap 4 of the cartridge lies on that side from which the tobacco smoke arrives and that the cartridge projects from the mouth piece 1 after it has been screwed off, so that the degree of exhaustion of the filter effected by the tobacco smoke may be quickly recognized from the coloration of the sealing cap. When being disposed accordingly, the filter when being examined needs not to be lifted from its place which always involves soiling the hands or any instruments used therefor. The cartridge is to fit tightly into the hollow chamber.

The filter material may be disposed either in layers of its particular components which, if desired, may be separated by easily permeable intermediate walls, or, alternatively, in a single composition of the particular components which form the filter material. The latter method has proved to be technically useful.

The grain size of the filter material may vary in a wide range; best results have been obtained by using a grain having a diameter of about 0.9 to 1.8 mm. Thus, beside a reasonable good filtering effect an unobstructed passage or flow of the smoke stream during the smoking process is obtained, which is still unrestrained even with strongly used and nearly exhausted filter cartridges.

The filter material may also be incorporated into the mouth piece of the cigarettes, cigarillos and cigars. However, this requires the use of a material having a grain size which is essentially smaller than that used in the mentioned cases. Here the grain size is preferably about 0.2 to 0.5 mm. in diameter.

The question as to whether smoking through the filter of this invention would result in any deterioration of the aroma has been carefully investigated, and it has been found useful or necessary respectively, to use special proportional amounts of the filter substances for binding the acid, basic and neutral components of the tobacco smoke, in order to provide a filter which does not deteriorate the aroma of the tobacco smoke and which nevertheless, effects a vigorous binding of the harmful components. It has been found that the filters of this invention even bring about an improvement of the tobacco smoke during smoking; for the scratching and acrid pungent taste caused in the mouth by smoking tobacco of minor quality may be prevented and a smoke which is well balanced, agreeable, under certain circumstances even mild may be obtained when smoking through the filters of this invention. On the basis of the results of the investigation the composition of the filter substances should be maintained within certain limits. In this connection it is essential that a more or less large excess of the cation exchange material over the other filter material described above (anion exchange material, organic bases on an adsorbent agent) should be always maintained. The following mixtures have proved to be advantageous: Three parts by weight of cation exchange material, 1 part 70 by weight of anion exchange material, and 1 part of adsorbent with a 1,2-aminoalcohol; or 4 parts by weight of cation exchange material, 1 part by weight of anion exchange material, 1 part by weight of adsorbent with a 1,2-aminoalcohol and 1 part of adsorbent with hydroxyl-

aminoacetate. A mixture consisting of 2 parts of sulfonated carbon which is sold under different trade names and which, in smaller grain sizes, is chiefly used for the purification of water, and of 1 part of activated carbon impregnated with 1-aminoethanol-2 has proved to be specially successful.

### EXAMPLE 1

#### *Impregnation of porous material with organic bases*

First, activated carbon (commercial) is tested by the following method as to its power of adsorption:

1 g. of activated carbon is shaken in a test tube with a red colored solution of 10 cc. water, 1 cc. of a 0.2% methyl red solution and 2 drops of 20% hydrochloric acid. Gradually, the color is to disappear and after 10 minutes the liquor, upon having been filtered, has to be totally colorless.

100 g. of an activated carbon fulfilling these conditions are intensely agitated or shaken with a solution, consisting of 200 cc. water and 2.5 cc. 1-aminoethanol-2 for about a quarter of an hour. Thereupon the solids are sucked off and slowly washed with about 1800 cc. of cold water. The last amount of water is to indicate only a weak alkaline reaction on indicator paper, corresponding to a pH of about 7.2 to 7.4. The activated carbon treated in this manner is dried in an evaporating dish on the water bath. This drying may be conducted more carefully in the vacuum.

When shaken with little cold water this reaction product should not indicate any alkaline reaction with indicator paper. However, when heating the aqueous mixture in a test tube until boiling a weak alkaline reaction will occur.

Alternatively, alcohol, acetone, ether, dioxane, or 35 acetonitrile may be used as diluent instead of water. The activated carbon with the material adsorbed thereon may also be prepared as described in Example 2.

In the same manner the activated carbon may be treated with the other mentioned organic bases, such as 40 e. g. phenylhydrazine, 1,2-ethylenediamine, 1,3-propylenediamine, 2-diethylaminoethanol, glucamine or a similar substance.

Alternatively, the porous materials mentioned above, such as e. g. cellulose, asbestos wool, plastic materials, 45 silica gel or a similar substance, may be used in the above example, instead of activated carbon.

In this case the following method may be used. The amine is first dissolved in a low boiling solvent or diluent. Thereupon the porous material is added to the solution 50 and the solvent or diluent is distilled off by heating the mixture on a water bath and applying a vacuum, if desired. Thus a uniform adsorption of the amine on cellulose, asbestos wool or any other porous material is effected. For instance, 1 g. of 1-ethylaminoethanol-2 is dissolved in 300 cc. ether and the solution obtained is added to 10 g. asbestos wool while well shaking. Thereupon the solvent is distilled off by heating the mixture on a water bath, thus leaving an asbestos wool which contains about 10% of 1-ethylaminoethanol-2 uniformly adsorbed thereon. The material thus obtained may be diluted, if desired, by mixing it in a ball mill with additional untreated asbestos wool to form a material with a lower content of 1-ethylaminoethanol-2.

### EXAMPLE 2

#### *Preparation of the filters*

In a glass tube 13 about 35 mm. long and 5 mm. in diameter provided with a perforated cap 14, as shown in Fig. 7, first 0.5 g. of a cation exchange material 15 is introduced, e. g. the commercially available product on the basis of sulfonated polystyrene resin (Amberlite IR-120), having a grain size of about 1.2 mm. The first layer is covered with a small, well permeable cotton wool stopper 16. Thereupon, 0.1 g. of an anion exchange mate-

rial 17 is introduced in the tube, e. g. the commercially available product derived from phenol-formaldehyde-amine resin having a grain size of 0.9 mm. After this layer has been covered again with a small, well permeable cotton wool stopper 18, 0.2 g. activated carbon 9, having a grain size of about 1.2 to 1.4 mm, and containing about 5% of di-2,2'-hydroxyethylamine adsorbed thereon, is introduced into the tube. The end of the tube is then sealed with a perforated cap 20.

In this case the activated carbon with the material adsorbed thereon is prepared as follows: 1 g. of di-2,2'-hydroxyethylamine is slowly added to 1 g. activated carbon while well stirring whereby the composition becomes warm. The moist paste obtained is further slowly mixed with 19 g. activated carbon while well stirring. There is thus obtained a homogeneous powder which does no longer smell of the added amine, is dry and may be stored for any desired length of time.

It was unexpected that the filter materials may be mixed with each other, for, because of the different properties of the cation and the anion exchange materials as well as of the organic bases it had to be assumed that they would affect each other when in mutual contact for a long time. Since, however, such action did not occur it was possible to use a substantially simpler process for the preparation of the filter. By means of a filling machine, e. g. a rotary filling apparatus, it is possible to exactly measure the ready mixtures consisting of the different filter materials and to quickly and continually fill them into the cartridge casings. Even the placing of the sealing cap and the sealing of the cartridge with adhesive or by means of heat treatment may be conducted automatically.

The mixtures of the filter materials may consist for instance of

I. 2 parts by weight of cation exchange materials (sulfonated carbon) and 1 part by weight of an adsorbent consisting of activated carbon with about 1% of 1-aminoethanol-2, or of

II. 2 parts by weight of cation exchange material (sulfonated carbon) and 1.5 parts by weight of an adsorbent consisting of activated carbon with about 0.75 or 1% or intermediate percentage amounts of 1-methylaminooethanol-2, or of

III. 3 parts by weight of cation exchange material (phenol sulfonic acid resin), 1 part by weight of anion exchange material (secondary amine on the basis of polystyrene) and 1 part by weight of an adsorbent consisting of activated alumina with about 5% of phenylhydrazine, or of

IV. 4 parts by weight of a cation exchange material (sulfonated carbon as used for the treatment of water), 1 part by weight of an anion exchange material (Amberlite IR-400, see U. S. Patent 2,591,573, a quaternary ammonium base with reduced basicity on the basis of polystyrene), 1 part by weight of an adsorbent consisting of silica gel with about 1% of semicarbazide and 1 part by weight of an adsorbent consisting of small paper balls with about 1% of glucamine, or, though less favorable, of

V. 2 parts by weight of an anion exchange material, e. g. Amberlite IR-413 (F. J. Myers, Eng. Ind. Chem. 35, 858 [1943]; R. Kunin and F. J. Myers, J. Amer. Chem. Soc. 69, 2874 [1947]) and 1 part by weight of an adsorbent consisting of asbestos wool which contains about 1% by weight of 1-benzylamino-ethanol-2.

### EXAMPLE 3

#### Test of the action of the new filters when compared with known filters

The test can be carried out according to the method which has been described by the inventors in the periodical "Arzneimittel-Forschung," vol. 4 (1954), pages 75-79.

The smoke, e. g. of a burning cigarette is passed through a filter which contains the substance to be tested

as to its detoxicating power, then the smoke is conducted through a tightly stuffed cotton wool column and finally through two washing bottles which are connected in series and which contain an *n*/1 or *n*/10 caustic soda solution and an *n*/1 or *n*/10 hydrochloric acid solution, the stream of smoke through the whole testing device being effected by means of the suction power of a water jet pump.

In order to obtain a good control of the smoke stream a round bottom flask with a stop cock is used which is connected between the water jet pump and the washing bottles. The speed of the stream is controlled so as to allow the burning of a cigarette to take place within about 6 to 8 minutes.

During the smoking process all tarry and less volatile substances, such as e. g. nicotine or other pyridine bases, aromatic compounds or a similar substance as far as they have passed the filter, are gathered in the cotton wool column, coloring the latter from a fair yellow to a deep dark brown. Those easily volatile components having acid properties are caught by the diluted caustic soda solution and those having basic properties are caught by the diluted hydrochloric acid. All components are determined by titration. The colored cotton wool column is extracted with ether in a Soxhlet apparatus. From the degree of coloration of the ether it is possible to determine even externally the more or less good effect of the filter. For a more exact test the ether solution is evaporated, strongly acidified with diluted sulfuric acid and titrated with an *n*/1 or *n*/10 solution of potassium permanganate at a temperature of 40° to 45° to reach the point, where after a reaction time of 1 minute the violet color of the permanganate solution remains stable. By this method of oxidation it is possible to clearly determine those organic materials which have passed the filter. For, the more cc. of the permanganate solution consumed (namely that number of cc. of the permanganate solution which is necessary to obtain a permanent violet coloration) the more of the harmful substances have unchangedly passed the filter into the cotton wool column which is connected downstream. Or, in short: the greater the number of consumed cc., the worse the filter.

The following table contains the results obtained with no filter used, with known filters and with the filters according to the invention.

TABLE  
[Comparison of the filter of this invention with known filters. The tests were carried out with the smoke of one cigarette per filter.]

| 50 | Filter cartridges                   | Visible degree of coloration of the cotton wool column | Consumption of                               |                        |                       |
|----|-------------------------------------|--------------------------------------------------------|----------------------------------------------|------------------------|-----------------------|
|    |                                     |                                                        | <i>n</i> /10 KMnO <sub>4</sub> solution, cc. | <i>n</i> /10 NaOH, cc. | <i>n</i> /10 HCl, cc. |
| 55 | without filter.....                 | +++++                                                  | 24.9                                         | 9.5                    | 0.5                   |
|    | silicagel.....                      | +++                                                    | 14.5                                         | 9.1                    | 0.0                   |
|    | activated carbon.....               | ++                                                     | 5.8                                          | 6.8                    | 0.0                   |
|    | filter cigarette of known type..... | ++                                                     | 3.8                                          | 9.5                    | 0.0                   |
| 60 | new filter of invention.....        | +                                                      | 1.0                                          | 4.8                    | 0.0                   |

The symbols + contained in the second column have the following meaning:

+++++=deep dark brown.

+++=dark brown.

+++=brown.

+++=light brown.

+++=yellow brown.

+=yellow.

0=colorless.

The filter of the invention used in the above comparison contained the following components: 2 parts by weight of sulfonated carbon and 1 part by weight of activated carbon with 1% of 1-aminoethanol-2.

### EXAMPLE 4

The good filtering effect was confirmed by an experiment with a person being very sensitive to nicotine when

smoking. While this person was able to smoke without any inconvenience a cigarette in a holder containing a filter in the form of a cartridge about 3.5 cm. long and about 0.5 cm. in diameter, filled with 0.5 g. sulfonated carbon (grain size 1.2 to 1.5 mm.) and with 0.25 g. carbon (an activated carbon described in "Die aktive Kohle" by O. Kausch, published by Wilhelm Knapp, Halle, Germany, 1928 and 1932) impregnated with 0.025 g. 1-aminoethanol-2, the same person when smoking a cigarette without this filter had to stop after a few puffs, because the known symptoms of supersensitivity to nicotine became extremely apparent.

We claim:

1. A tobacco smoke filter comprising a chamber adapted to afford passage of tobacco smoke therethrough containing granular ion exchange material, a granular porous substance and a difficultly volatile amino compound adapted to react with organic carbonyl compounds to form a non-volatile product adsorbed on said granular porous substance.

2. A tobacco smoke filter comprising a chamber adapted to afford passage of tobacco smoke therethrough containing a mixture comprising granular ion exchange material, a granular porous substance and a difficultly volatile amino compound adapted to react with organic carbonyl compounds to form a non-volatile product adsorbed on said granular porous substance.

3. A tobacco smoke filter comprising a chamber adapted to afford passage of tobacco smoke therethrough containing granular ion exchange material, a granular porous substance and a difficultly volatile amino compound adapted to react with organic carbonyl compounds to form a non-volatile product adsorbed on said granular porous substance in a quantity of about 0.1% to about 10% calculated on the weight of the porous substance.

4. A tobacco smoke filter comprising a chamber adapted to afford passage of tobacco smoke therethrough containing a mixture comprising a granular ion exchange material, a granular porous substance and a difficultly volatile amino compound adapted to react with organic carbonyl compounds to form a non-volatile product adsorbed on said granular porous substance in a quantity of about 0.1% to about 10% calculated on the weight of the porous substance.

5. A tobacco smoke filter comprising a chamber adapted to afford passage of tobacco smoke therethrough containing a mixture comprising a granular cation exchange material and a granular porous substance having absorbed thereon a difficultly volatile amino compound adapted to react with organic carbonyl compounds to form a non-volatile product in a quantity of about 0.1% to about 10% calculated on the weight of the porous substance.

6. A tobacco smoke filter comprising a chamber adapted to afford passage of tobacco smoke therethrough containing a mixture comprising a granular cation exchange material and a granular porous substance having absorbed thereon a difficultly volatile amino compound adapted to react with organic carbonyl compounds to form a non-volatile product in a quantity of about 0.1% to about 10% calculated on the weight of the porous sub-

stance, and in which mixture the quantity of the granular cation exchange material is in excess over the quantity of the granular porous substance containing the adsorbed amino compound.

5 7. A tobacco smoke filter comprising a chamber adapted to afford passage of tobacco smoke therethrough containing a mixture of two parts by weight of a granular sulfonated carbon with one part by weight of a granular activated carbon which has adsorbed about one percent of 1-aminoethanol-2.

10 8. A tobacco smoke filter comprising a chamber adapted to afford passage of tobacco smoke therethrough containing a mixture of two parts by weight of a granular sulfonated carbon with 1.5 parts by weight of a granular activated carbon which has adsorbed about 0.75% to 1% of 1-methylaminoethanol-2.

15 9. A tobacco smoke filter comprising a chamber adapted to afford passage of tobacco smoke therethrough containing a mixture of three parts by weight of a granular phenol sulfonic acid resin material with one part by weight of a granular anion-exchange polystyrene compound and with one part by weight of a granular activated alumina material which has adsorbed about 5% of phenylhydrazine.

20 10. A tobacco smoke filter comprising a chamber adapted to afford passage of tobacco smoke therethrough containing a mixture of two parts by weight of a granular sulfonated carbon with one part by weight of a granular activated carbon which has adsorbed about one percent of 1-aminoethanol-2 and wherein the granular particles have a diameter of from 0.9 mm. to 1.8 mm.

25 11. A tobacco smoke filter comprising a chamber adapted to afford passage of tobacco smoke therethrough containing a mixture of two parts by weight of a granular sulfonated carbon with 1.5 parts by weight of a granular activated carbon which has adsorbed about 0.75% to 1% of 1-methylaminoethanol-2 and wherein the granular particles have a diameter of from 0.9 mm. to 1.8 mm.

30 12. A tobacco smoke filter comprising a chamber adapted to afford passage of tobacco smoke therethrough containing a mixture of three parts by weight of a granular phenol sulfonic acid resin material with one part by weight of a granular anion-exchange polystyrene compound and with one part by weight of a granular activated alumina material which has adsorbed about 5% of phenylhydrazine and wherein the granular particles have a diameter of from 0.9 mm. to 1.8 mm.

35 13. A tobacco smoke filter comprising a cylindrical cartridge perforated at both ends containing granular ion exchange material, a granular porous substance and a difficultly volatile amino compound adapted to react with organic carbonyl compounds to form a non-volatile product adsorbed on said granular porous substance.

#### 55 References Cited in the file of this patent

##### FOREIGN PATENTS

|         |               |               |
|---------|---------------|---------------|
| 337,200 | Great Britain | Oct. 30, 1930 |
| 497,708 | Great Britain | Dec. 19, 1938 |
| 501,402 | Belgium       | Mar. 15, 1951 |